

F. M. RUSCHHAUPT,  
ROOFING SHINGLE,  
APPLICATION FILED MAY 31, 1913.

1,197,307.

Patented Sept. 5, 1916.

*Fig. 1.*



*Fig. 2.*



*Fig. 3.*



Witnesses  
C. H. Hermich  
Ruth Ringle

Attentor  
Frederick M. Ruschhaupt  
by Gilliom & Gilliom atqrs.

# UNITED STATES PATENT OFFICE.

FREDERICK M. RUSCHHAUPT, OF MILWAUKEE, WISCONSIN, ASSIGNOR TO AMERICAN FLEXIBLE SLATE AND COVERING CO., OF MILWAUKEE, WISCONSIN, A CORPORATION OF WISCONSIN.

## ROOFING-SHINGLE.

1,197,307.

Specification of Letters Patent. Patented Sept. 5, 1916.

Application filed May 31, 1913. Serial No. 770,973.

To all whom it may concern:

Be it known that I, FREDERICK M. RUSCHHAUPT, a citizen of the United States, and resident of Milwaukee, county of Milwaukee, 5 and State of Wisconsin, have invented certain new and useful Improvements in Roofing-Shingles, of which the following is a specification and which are illustrated in the accompanying drawings, forming a part 10 thereof.

The invention relates to shingles for covering roofs, and the like, and has for its object to provide a shingle which will effectively serve to resist abrasion by wear or by 15 the action of the weather, which shall be substantially fireproof, and which may be inexpensively produced and applied to either flat, curved, or angular surfaces.

The invention contemplates a shingle produced wholly from plastic materials without the use of any fabric or sheet material as a reinforcement, as from the composition of matter disclosed in Patent No. 1,051,769, issued to my assignee, American Flexible 25 Slate and Covering Co., on January 28th, 1913.

In the accompanying drawings, Figures 1 and 2 are perspective views showing sheets of two different forms which may be provided by the invention; and Fig. 3 is a diagrammatic view illustrating a step in a process which may be used for producing sheets of the form illustrated in Fig. 2.

The shingle forming the subject of this 35 invention is produced by rolling a plastic material consisting of a mineral powder formed into a homogeneous dough-like mass, by mixing therewith suitable quantities of a viscous material, such as the pitch or tar 40 produced from the distillation of coal or gum asphalt or asphaltic tar, or mixtures of these substances. If desired a suitable coloring matter or surfacing material may be applied to the mass during the rolling 45 operation, for varying the color or character of the surface of the sheet.

The shingles are desirably produced at a low cost by the use of inexpensive materials, preferably those which may be obtained in 50 any locality. I have found that shingles of very good quality may be produced by using thoroughly sifted ash from anthracite coal as the principal powdered mineral constituent, and by the use of coal tar pitch and coal 55 tar as the principal constituents of the viscous material. One formula principally

containing these materials and serving to produce desirable sheets is that described in my said Patent No. 1,051,769 as follows:

|                                                                                               |           |    |
|-----------------------------------------------------------------------------------------------|-----------|----|
| Coal tar pitch-----                                                                           | 18 pounds | 60 |
| Coal tar-----                                                                                 | 9 pounds  |    |
| Gum asphalt-----                                                                              | 7 pounds  |    |
| Asphaltic tar or oil-----                                                                     | 4 pounds  |    |
| Ash, preferably from anthracite coal-----                                                     | 40 pounds | 65 |
| Sand-----                                                                                     | 10 pounds |    |
| Portland cement-----                                                                          | 6 pounds  |    |
| Fiber, of either an organic or inorganic fibrous substance but preferably asbestos fiber----- | 3 pounds  | 70 |
| Alum, or aluminum-sulfate or ammonium-sulfate-----                                            | 3 pounds  |    |

In using the above formula I have found it desirable to thoroughly mix the dry constituents and viscous constituents separately, the viscous constituents being then added to the dry materials and the whole mass thoroughly mixed and kneaded at a suitable temperature, as in a steam jacketed mixing 75 vessel. It will be understood that to enable the viscous materials to be thoroughly mixed with each other and with the dry materials, it is necessary that they first be melted, in accordance with the usual practice of working such materials.

The mass produced from the use of the formula above mentioned has a dough-like consistency when warm, and may be readily rolled out into sheets, of any desired size 90 and thickness, from which the shingles, as 10 (Fig. 1) may be cut. Shingles so formed are tough and but slightly flexible at the ordinary temperature. If warmed to a temperature of 100 degrees Fahrenheit, they 95 may be formed to any desired shape, as for fitting them into the gutters or over the ridges of roofs and the like. If desired shingles of the form shown at 11 (Fig. 2) and having the well known wedge shape 100 form of wooden shingles may be produced. Shingles of the form shown at 10 (Fig. 1) or at 11 (Fig. 2) may be laid upon the roof in the same manner as wooden shingles. However, in covering a roof with such 105 shingles the use of tin or other sheet metal in the gutters, and the like, is unnecessary as the shingles herewith provided may be readily fitted into such parts of the roof and effectively serve as a protection against the 110 weather.

Sheets of the form shown at 11 (Fig. 2)

are conveniently produced by rolling the before mentioned plastic material between rolls, as 12, 13, (Fig. 3). For this purpose one of the rolls, as 13, is eccentrically mounted and is preferably of such size as to have a circumference equal to twice the length of the finished shingle. If a quantity of the material, as 14, which has previously been reduced by rolling to the form of a sheet 10 having approximately the thickness of the thicker end of the shingle, be fed to these rolls while still warm, it will issue from the rolls in the form of a sheet 15 of gradually varying thickness, the amount of variation 15 in thickness being determined by the eccentricity of the roll 13. Obviously this may be varied to produce the degree of taper desired in the finished shingles. The shingles 11 are completed by cutting the sheet 15 20 transversely at the points of its greatest and least thicknesses, as at 16 and 17 (Fig. 3).

If a colored or hardened surface is desired upon the shingles, a finely powdered or granulated material will be sifted upon the 25 surface of the unfinished sheet, as 14, immediately prior to its passage through the finishing rolls, as 12, 13. A desirable surface color is produced by sifting finely powdered red oxid of iron upon the surface 30 of the unfinished sheet, as 14. The character of the surface may be varied by the use of such substances as fine gravel, crushed mica, slate, or burnt clay product, in a manner similar to that described for the red

oxid of iron. In either case the surface of 35 the shingle becomes thoroughly impregnated with the coloring or crushed material, and a permanent product is produced. It will be understood that shingles of either of the forms shown at 10, (Fig. 1) or 11 (Fig. 2) 40 may be produced with such modified surfaces.

In applying the shingles to a roof they will be secured in place with nails and overlapped after the manner of laying 45 ordinary wooden shingles. The character of the sheets is such as to effectively resist the action of the weather and wear, as also the action of acids or alkaline and abrasive cleansing materials. Furthermore, while the 50 shingles contain a small proportion of combustible materials, these are of a character which are ignited with difficulty, and they constitute such an inconsiderable proportion of the entire mass that the shingles are substantially fireproof. Their ignition is effected with such difficulty that they serve to 55 thoroughly protect a structure against fire by ignition of the roof covering.

I claim as my invention—

A homogeneous pliable rolled roofing shingle comprising a large proportion of finely divided incombustible material and a viscous binder.

FREDERICK M. RUSCHHAUPT.

Witnesses:

E. J. GROSS,  
MAE TRAPSHUH.